

M. E. RAUSCH.  
METHOD FOR TREATING EMERY WHEELS.  
APPLICATION FILED OCT. 20, 1917.

1,278,214.

Patented Sept. 10, 1918.

Fig. 1



Fig. 2



Inventor

Mathew C. Rausch  
By Watson E. Coleman

Attorney

# UNITED STATES PATENT OFFICE.

MATHEW C. RAUSCH, OF JACKSON, MICHIGAN.

## METHOD FOR TREATING EMERY-WHEELS.

1,278,214.

Specification of Letters Patent. Patented Sept. 10, 1918.

Application filed October 20, 1917. Serial No. 197,647.

To all whom it may concern:

Be it known that I, MATHEW C. RAUSCH, a citizen of the United States, residing at Jackson, in the county of Jackson and State 5 of Michigan, have invented certain new and useful Improvements in Methods for Treating Emery-Wheels, of which the following is a specification, reference being had to the accompanying drawings.

10 This invention relates to certain improvements in methods for treating emery stone, and it is an object of the invention to provide a novel and improved method whereby the binding material is transformed from its 15 native hardness or rigidity to such a degree of softness that the emery stone can be bored by an ordinary steel or iron drill.

It is also an object of the invention to provide a novel and improved method of 20 treating emery stone or more particularly emery whereby a grinding wheel may be produced which is provided with an internal grinding surface.

In the accompanying drawings:

25 Figure 1 is a diagrammatic view illustrating the first step in my improved method; and

Fig. 2 is a diagrammatic view illustrating a further step employed in my improved 30 method.

In my improved method to treat emery stone in order to permit the same to be drilled or bored I first place the emery stone in a solution of one part of soda ash to five 35 parts of water. The emery stone is submerged in this solution for sixty hours and then a second solution is added to the first named solution and said second solution comprises two parts of lye to three parts of 40 water. After the second solution has been added the temperature is brought to a heat of 60° F. and the emery stone is immersed in this combined solution and at this temperature for one hour. The combined solution 45 is then permitted to cool until the temperature thereof is reduced to 20° F. The emery stone is operated upon while still in the solution because the particles which are loosened by the solution do not reset. The loosened

particles are freed from the article produced by rotating the same at a minimum rotation of substantially ten thousand revolutions per minute.

My improved method is particularly adapted for use in the production of grinding wheels provided with internal grinding surfaces and the operations on the emery stone while in the combined solution consists in the requisite dressing of the surface of the emery wheel and boring or drilling therethrough an opening 1. The opening 1 results in an annular internal grinding surface 2 which may be effectively employed for grinding purposes and in a manner which is well known to those skilled in the 65 use of emery wheels.

A further advantage possessed by my improved method is the facility and convenience with which used emery wheels of the ordinary type may be treated in order 70 to produce an internal grinding surface 2 whereby the life of such emery wheel may be materially prolonged and whereby a material saving of the emery is effected.

The method hereinbefore set forth particularly relates to emery of "number seven" grade which is the hardest grade of emery. In treating the lower or softer grades of emery wheels the solutions are weakened and the degrees of heat lowered and also the 80 length of time of immersion is shortened.

I claim:

The method of treating an emery stone which consists in subjecting the stone to a relatively dilute alkaline solution at ordinary temperature, then subjecting the stone to a more concentrated alkaline solution at a higher temperature, then mechanically operating upon the stone while in said last mentioned solution to remove material therefrom, and then rotating the stone.

In testimony whereof I hereunto affix my signature in the presence of two witnesses.

MATHEW C. RAUSCH.

Witnesses:

JACOB FREY,  
HUGO C. LOESER.